

## 1

2,993,007

**N-ALKYLHETEROCYCLIC NITROGEN-CONTAINING DERIVATIVES AS CORROSION-INHIBITORS**  
 Donald L. Andersen, Minneapolis, Minn., and Peter E. Throckmorton, Manhattan, Kans., assignors to General Mills, Inc., a corporation of Delaware  
 No Drawing. Filed Mar. 8, 1957, Ser. No. 644,751  
 3 Claims. (Cl. 252—392)

This invention relates to the use of N-alkylheterocyclic compounds as corrosion inhibitors. More specifically, this invention relates to their use as corrosion inhibitors in static water and boiler water.

Corrosion of metallic substances represents a major industrial problem. Every year the loss to industry through corrosion amounts to millions of dollars. In general, this corrosion takes place when the metallic substances, especially ferrous-containing metals, come in contact with a watery media, i.e., water, aqueous solutions, water vapor and the like. Various methods are presently known and utilized for preventing or inhibiting the corrosive activity of the various aqueous media. The most frequently employed method for inhibiting and preventing corrosion is to cover the surface of the metallic substance with a protective coating.

It has now been discovered that a tenacious protective film of essentially monomolecular dimensions is formed when N-alkylheterocyclic compounds are contacted with the surface of the metallic substance. This film, as utilized in steam condensate lines, in addition to forming a protective coating over the surface, has a surface activity that maintains the heat transfer efficiency of the lines at their optimum.

Suitable compounds are represented by the general formula



where R is a straight chained hydrocarbon radical, and T is hydrogen or a lower alkyl radical. Preferably, T represents hydrogen and R represents an aliphatic hydrocarbon radical corresponding to the chain length of fatty acids in coconut oil, i.e., "coco," since these compounds are more effective than the other members of this class of compounds. It is noted that the heterocyclic nucleus in the above compounds is saturated, has a long chained aliphatic hydrocarbon radical attached to the nitrogen member of the ring, and the heterocyclic ring contains at least two dissimilar atoms other than carbon. These features are the salient characteristics of the compounds which are the exceptional corrosion inhibitors of this invention as will be shown hereinafter.

Thus, an object of this invention is to teach a family of compounds which possess an unusually high degree of effectiveness in divers corrosion inhibiting problems.

Another object of this invention is to teach a family of compounds which are more effective than presently employed compounds.

Specifically, in regard to protection of steam lines the compounds of this invention have sufficient steam volatility such that adequate quantities of the compounds are entrained in the steam to act as corrosion inhibitors in condensate return lines.

Furthermore, the salts of these compounds are liquids at room temperature. As such they may be metered directly as 100% active liquids without any trouble which greatly facilitates their ease of handling. This fact obviates any need for the preparation of stock solutions for sale to consumers and directly decreases freight charges in shipments to the consumer.

## 2

Other objects and advantages to this invention will become obvious upon reading the subsequent portions of the specification.

## EXAMPLE I

The "static" water test and "dynamic" water test were employed to evaluate the effectiveness of the various compounds. The data obtained in these tests are empirical accelerated laboratory tests in which the corrosion effect is multiplied many times. For instance, in actual practice the systems would be closed systems whereas in the "dynamic" water test fresh air is constantly admitted into the system. The procedures followed in these tests are as follows:

## Static water test

*Step A.*—1" × 1" × 1/16" S.A.E. 1020 mild steel coupons having a 5/32" diameter hole were pickled as follows:

- (1) soak coupons in reagent grade acetone and dry in air.
- (2) pickle 10.0 min. in concentrated HCl at room temperature with agitation.
- (3) rinse in distilled water, acetone dip, dry at reduced pressure in desiccator and weigh to ±0.0002 gm. immediately.

*Step B.*—Suspend each coupon from a Pyrex hook in 150 ml. ± ml. of test solution (prepared from distilled water to ±1 p.p.m. inhibitor based on 100% active material) and control (distilled water) so as to be fully immersed with the coupon's top edge 1/8" to 3/8" below test solution surface using 250 ml. Pyrex Erlenmeyer flasks as a test container.

*Step C.*—Leave the coupon suspended for 7 days ±2 hours at room temperature.

*Step D.*—Remove coupons from test flasks and soak in inhibited 5% HCl at ambient temperature for 5.0 minutes to loosen scale.

*Step E.*—Lightly scrub each coupon with soft bristle brush and commercial-type detergent cleanser to completely remove corrosion products, but no base metal.

*Step F.*—Rinse coupons with distilled water, then acetone; dry at reduced pressure in desiccator and reweigh immediately.

*Step G.*—Calculate percent inhibition according to the following formula:

$$\frac{\sum_{i=1}^{i=n_c} C_i - \sum_{i=1}^{i=n_t} t_i}{\sum_{i=1}^{i=n_c} C_i} \times 100\%$$

i=individual test value

n=number of individual test values

c=percent weight loss of control coupon (identical test with no inhibitor present)

t=percent weight loss of test coupon

## Dynamic test

Steps A and B are the same as in the static water test.

*Step C.*—Place 1000 ml. of test sample or control (distilled water) in a large round bottomed Pyrex flask used as a boiler pot and 500 ml. in the test chamber (500 ml. Pyrex Erlenmeyer flask) containing 3 coupons totally submerged and suspended from Pyrex hooks and adjust the test chamber so that this liquid level will be maintained with the overflow returning to the boiler pot.

*Step D.*—Heat the boiler pot so as to effect the steam distillation.

*Step E.*—Condense the steam and allow the condensate to enter the test chamber which is maintained at a temperature of 25 to 28° C.



from coconut fatty acids and forming a protective film  
on the metallic substances with said compound.

References Cited in the file of this patent

UNITED STATES PATENTS

2,239,841 Cook Apr. 29, 1941  
2,597,260 Reck May 20, 1952

2,692,879 Hales Oct. 26, 1954  
2,773,879 Sterlin Dec. 11, 1956  
2,829,945 Krieg Apr. 8, 1958  
2,850,461 Bloch et al. Sept. 2, 1958

FOREIGN PATENTS

Great Britain Nov. 18, 1935